# EUROPEAN PATENT SPECIFICATION

(11) **EP 0 830 941 B1**
(45) Date of publication and mention of the grant of the patent: **02.07.2003**
(21) Application number: 97202780.9
(22) Date of filing: 10.09.1997
(51) Int. Cl.: B41C 1/10, B41M 5/40

(54) **A heat mode recording material and method for producing driographic printing plates**
Im wärmeverfahren arbeitendes Aufzeichnungsmaterial und Verfahren zur Herstellung von Druckplatten, welche kein Anfeuchtwassen benötigen
Matériau d'enregistrement thermosensible et procédé pour la production de plaques lithographiques à sec

(30) Priority: 18.09.1996 EP 96202603
(43) Date of publication of application: 25.03.1998
(73) Proprietor: AGFA-GEVAERT, 2640 Mortsel (BE)
(72) Inventor: Verschueren, Eric, 2640 Mortsel (BE); Vermeersch, Joan, 2640 Mortsel (BE); Van Trier, Jean, 2640 Mortsel (BE)

(56) References cited:
- EP-A- 0 598 544
- EP-A- 0 620 502
- EP-A- 0 698 822
- EP-A- 0 713 140
- EP-A- 0 727 714
- US-A- 4 583 103
- US-A- 5 198 408
- DATABASE WPI Section Ch, Week 9324 Derwent Publications Ltd., London, GB; Class A97, AN 93-191182 XP002028577 & JP 05 116 474 A (OJI PAPER CO) , 14 May 1993
- DATABASE WPI Section Ch, Week 8311 Derwent Publications Ltd., London, GB; Class A97, AN 83-26423K XP002028578 & JP 58 020 495 A (RICOH KK) , 5 February 1983

## Description

### 1. Field of the invention.

The present invention relates to a heat mode recording material for making a lithographic printing plate for use in lithographic printing without dampening. The present invention further relates to a method for imaging said heat mode recording material by means of a laser.

### 2. Background of the invention.

Lithographic printing is the process of printing from specially prepared surfaces, some areas of which are capable of accepting ink (oleophilic areas) whereas other areas will not accept ink (oleophobic areas). The oleophilic areas form the printing areas while the oleophobic areas form the background areas.

Two basic types of lithographic printing plates are known. According to a first type, so called wet printing plates, both water or an aqueous dampening liquid and ink are applied to the plate surface that contains hydrophilic and hydrophobic areas. The hydrophilic areas will be soaked with water or the dampening liquid and are thereby rendered oleophobic while the hydrophobic areas will accept the ink. A second type of lithographic printing plates operates without the use of a dampening liquid and are called driographic printing plates. This type of printing plates comprise highly ink repellant areas and oleophilic areas. Generally the highly ink repellant areas are formed by a silicon layer.

Driographic printing plates can be prepared using a photographic material that is made image-wise receptive or repellant to ink upon photo-exposure of the photographic material. However heat mode recording materials, the surface of which can be made image-wise receptive or repellant to ink upon image-wise exposure to heat and/or subsequent development are also known for preparing driographic printing plates.

For example in DE-A-2512038 there is disclosed a heat mode recording material that comprises on a support carrying or having an oleophilic surface (i) a heat mode recording layer containing a self oxidizing binder e.g. nitrocellulose and a substance that is capable of converting radiation into heat e.g. carbon black and (ii) a non-hardened silicon layer as a surface layer. The disclosed heat mode recording material is image-wise exposed using a laser and is subsequently developed using a developing liquid that is capable of dissolving the silicon layer in the exposed areas. Subsequent to this development the silicon surface layer is cured. Due to the use of naphta as a developing liquid the process is ecologically disadvantageous. Further since the surface layer is not hardened the heat mode recording material may be easily damaged during handling.

FR-A-1.473.751 discloses a heat mode recording material comprising a substrate having an oleophilic surface, a layer containing nitrocellulose and carbon black and a silicon layer. After image-wise exposure using a laser the imaged areas are said to be rendered oleophilic. The decomposed silicon layer is not removed. Ink acceptance of the obtained plates is poor and the printing properties such as printing endurance and resolution of the copies is rather poor.

Research Disclosure 19201 of april 1980 discloses a heat mode recording material comprising a polyester film support provided with a bismuth layer as a heat mode recording layer and a silicon layer on top thereof. The disclosed heat mode recording material is imaged using an Argon laser and developed using hexane.

EP-A-573091 discloses a method for making a lithographic printing plate requiring a heat mode recording material comprising on a support having an oleophilic surface (i) a recording layer having a thickness of not more than 3µm and containing a substance capable of converting the laser beam radiation into heat and (ii) a cured oleophobic surface layer and wherein said recording layer and oleophobic surface layer may be the same layer.

EP-A-698 822 discloses a lithographic printing plate precursor having a flexible support carrying a surface capable of being differentiated in ink accepting and ink repellant areas upon imagewise exposure, and an optional development step, characterised in that said flexible support is a polyester film having a thickness between 0.075 mm and 0.35 mm and consisting of at least 75% by weight of polyethylene naphthalene dicarboxylate. A method of making a lithographic printing plate from said precursor, by exposure and optional development, is also described.

JP-A-5116474 describes a planographic printing form sheet, typically for use in xerography, which comprises a paper base material and waterproof layers formed on both sides of the base, one such surface carrying a layer comprising zinc oxide and a binder resin, the other surface having a layer comprising inorganic pigment and a binder resin. The sheet may be made up by either thermal image transfer or electrostatic image transfer and may then be fed to a printer in sheetwise manner in view of the low friction coefficient of the printed layer to the back layer.

JP-A-58020495 discloses a lithographic printing master, again useful in e.g. xerography, comprising a support coated on the front side with a precoat layer, an optional water-resistant layer and a photosensitive layer comprising a zinc oxide-resin dispersion system and, on the back side, with a conducting treatment layer containing a pigment mixture of clay with calcium carbonate and/or zinc oxide, a binder comprising weakly anionic or non-ionic emulsion resin, cationic and polymeric electrolyte and wax emulsion. The printing master benefits from high temperature storage stability and low tendency to stain on rubbing, in addition to having a friction coefficient suitable to prevent slipping on transferring."

From the above it can be seen that a number of proposals have been made for making a driographic printing plate using a heat mode recording material. All these plates have the disadvantage that they exhibit blocking. This results in difficulties in all steps wherein said materials are transported such as the winding-up during the fabrication, the format cutting and the packaging, the automatic loading on the press, the transport through the irradiation station, etc.,

### 3. Summary of the invention.

According to the present invention it is an object to provide an alternative heat mode recording material for making a driographic printing plate of high quality that exhibits less blocking.

It is a further object of the present invention to provide a method for obtaining a driographic printing plate of high quality using a heat mode recording material that exhibits less blocking.

Further objects of the present invention will become clear from the description hereinafter.

According to the present invention there is provided a heat mode recording material comprising on a flexible support having an oleophilic surface (i) a recording layer containing a light-to-heat converting substance capable of converting radiation into heat and (ii) an oleophobic surface layer, wherein said oleophobic surface layer and said recording layer may be the same layer, characterized in that the recording material comprises a back side coating and/or that a matting agent is present in the oleophobic surface layer, and further characterized in that the kinetic coefficient of friction (µₖ) of said material when sliding one side of said material over the other side of said material is not more than 2.6.

According to the present invention there is also provided a method for making a lithographic printing plate requiring no dampening liquid comprising the steps of:
- image-wise exposing by means of a laser beam a heat mode recording material according as described above
- developing the exposed heat mode recording material thereby removing said oleophobic surface -layer-in-the-exposed areas so that the underlying oleophilic surface is exposed.

### 4. Detailed description of the invention.

It has been found that the above described heat mode recording material exhibits a lowered blocking when the kinetic coefficient of friction is not more than 2.6, what leads to an easier production and use of said material and to printing plates which are improved in regard to their physical properties (less wrinkles) The kinetic coefficient of friction (µₖ) is measured according to the norm ASTM D1894 whereby the heat mode recording materials are so placed that the back side of the underlying material is in contact with the front side of the upperlying material. With back side of said material is meant that side of the material in regard to the flexible support which does not carry the oleophobic surface layer where with front side is meant that side of the material in regard to the flexible support that carries the oleophobic surface layer.

Preferably the kinetic coefficient of friction (µₖ) is not higher than 1.25. The lower limit should be as low as possible but is for practical reasons preferably not lower than 0.05, more preferably not lower than 0.10.

In order to lower the kinetic coefficient of friction the flexible support of the heat mode recording material is treated with a back side coating or there is added a matting agent to the oleophobic surface layer or both methods are used together.

A preferred back side coating according to the invention contains between 175 and 750 mg/m² gelatin, between 50 and 1000 mg/m² colloidal silica with a surface area of at least 100 m²/gr, more preferably at least 300 m²/gr and between 1 and 100 mg/m² of amorphous silica, preferably with a diameter between 1 and 10 µm.

Another preferred back side coating according to the invention comprises between 100 and 500 mg/m² of a polymethyl-methacrylate latex (particles diameter preferably between 25 and 300 nm), between 5 and 50 mg/m² colloidal silica with a surface area of at least 100 m²/gr, between 3 and 30 mg/m² of a polyethylene wax, between 3.1 and 12 mg/m² of polystyrene sulphonic acid, between 0.9 and 4 mg/m² of poly(3,4-ethylenedioxy-thiophene) and between 10 and 100 mg/m² of polymethyl-methacrylate matting agent (preferably with a diameter between 2 and 10 µm).

Still another preferred back side coating according to the invention comprises PVA, TiO₂ and hydrolyzed tetraalkyl orthosilicate, wherein SiO₂ constitutes between 7 and 30 weight % of the total weight of said matrix, TiO₂ constitutes between 63 and 83 weight % of the total weight of said matrix and PVA constitutes between 7 and 30 weight % of the total weight of said matrix. The total weight of said matrix lies between 5 and 10 g/m². To said matrix can be added in an amount between 3 and 500 mg/m² a matting agent such as starch, silicium oxide, silicates, glass pearls, toner particles.

A matting agent added to the oleophobic surface layer in order to lower the kinetic coefficient of friction may be an organic polymer or copolymer such as a copolymer of acrylic acid and methyl acrylate or a copolymer of styrene, methyl-methacrylate and maleic acid. More preferably said matting agent is an inorganic compound such as silica or a silicate.

Said matting agent has a weight average diameter of at least 2 µm, more preferably of at least 3 µm, most preferably of at least 4 µm. The maximum weight average is not so important but is for practical reasons less than 100 µm, more preferably less than 60 µm.

In accordance with the invention said oleophobic surface layer preferably comprises at least 30mg/m² of a matting agent with a weight average diameter of at least 2 µm, more preferably between 50 and 500 mg/m² of said matting agent, most preferably between 75 and 300 mg/m² of said matting agent.

Flexible supports suitable for use in accordance with the present invention may be opaque or transparent, e.g. a paper support or resin support. When a paper support is used preference is given to one coated at one or both sides with an Alpha-olefin polymer, e.g. a polyethylene layer which optionally contains an anti-halation dye or pigment. It is also possible to use an organic resin support e.g. cellulose nitrate film, cellulose acetate film, poly(vinyl acetal) film, polystyrene film, poly(ethylene terephthalate) film, poly(ethylene naphthalenedicarboxylate) film, polycarbonate film, polyvinylchloride film or poly-Alpha-olefin films such as polyethylene or polypropylene film. The thickness of such organic resin film is preferably comprised between 0.06 and 0.35 mm. These organic resin supports are preferably coated with a oleophilic adhesion layer.

According to a preferred embodiment of the present invention the heat mode recording material contains a separate heat mode recording layer containing the heat converting substance comprised between the support and the oleophobic surface layer. Examples of substances capable of converting radiation into heat are e.g. carbon black, infrared or near infrared absorbing dyes or pigments, metals such as Bi, Sn, Te etc. or a combination thereof. Suitable infrared dyes are disclosed in e.g. US-4833124, EP-321923, US-4772583, US-4942141, US-4948776, US-4948777, US-4948778, US-4950639, US-4950640, US-4912083, US-4952552, US-5024990, US-5023229 etc.. Suitable infrared pigments are e.g. HEUCODOR metal oxide pigments available from Heubach Langelsheim. When a metal such as e.g. bismuth is used as a heat converting substance the recording layer is preferably a vacuum deposited metal layer.

According to the present invention the thickness of the recording layer is preferably not more than 3µm in order to obtain a printing plate of acceptable quality, more preferably the thickness will be less than 2.5µm. Typically the recording layer preferably has a thickness between 15 nm and 1.5µm. The preferred maximum thickness of 3µm of the recording layer is especially important when exposure is carried out through the support.

According to a particular embodiment of the present invention the recording layer may be a vacuum deposited aluminium layer. The thickness of such an aluminium layer however should be less than 25 nm and more preferably between 10 nm and 22,5 nm. When the thickness of the aluminium recording layer becomes too large the heat mode recording material in connection with the present invention cannot be imaged.

The heat mode recording layer used in connection with the present invention may contain a binder e.g. gelatin, cellulose, cellulose esters e.g. cellulose acetate, nitrocellulose, polyvinyl alcohol, polyvinyl pyrrolidone, a copolymer of vinylidene chloride and acrylonitrile, poly(meth)acrylates, polyvinyl chloride, silicone resin etc.. The recording layer may further contain other ingredients such as e.g. wetting agents, matting agents, anti-oxidizing agents etc.. Preferably the heat mode recording layer contains a polymer containing covalently bound chlorine. Alternatively part or all of this polymer may be contained in a separate layer located adjacent to the heat mode recording layer and most preferably between the support and the heat mode recording layer.

The heat mode recording layer in connection with the present invention may be hardened. For example a nitrocellulose layer hardened with an isocyanate or a melamine may be used.

It has been found that when a polymer containing covalently bound chlorine is contained in the heat mode recording layer of a recording material or in an adjacent layer the speed of the recording material can be improved.

Suitable chlorine containing polymers for use in accordance with the present invention are e.g. polyvinyl chloride, polyvinylidene chloride, a copolymer of vinylidene chloride, an acrylic ester and itaconic acid, a copolymer of vinyl chloride and vinylidene chloride, a copolymer of vinyl chloride and vinyl acetate, a copolymer of butylacrylate, vinyl acetate and vinyl chloride or vinylidene chloride, a copolymer of vinyl chloride, vinylidene chloride and itaconic acid, a copolymer of vinyl chloride, vinyl acetate and vinyl alcohol, chlorinated polyethylene, polychloroprene and copolymers therof, chlorosulfonated polyethylene, polychlorotrifluoroethylene, polymethyl-alpha-chloroacrylate etc.

The chlorine containing polymer used in connection with the present invention may be prepared by various polymerization methods of the constituting monomers. For example, the polymerization may be conducted in aqueous dispersion containing a catalyst and activator, e.g., sodium persulphate and meta sodium bisulphite, and an emulsifying and/or dispersing agent. Alternatively, the homopolymers or copolymers used with the present invention may be prepared by polymerization of the monomeric components in the bulk without added diluent, or the monomers may be reacted in appropriate organic solvent reaction media. The total catalyst-activator concentration should generally be kept within a range of about 0.01% to about 2.0% by weight of the monomer charge, and preferably within a range of concentration of 0.1% to 1.0%. Improved solubility and viscosity values are obtained by conducting the polymerization in the presence of mercaptans such as ethyl mercaptan, lauryl mercaptan, tertiary dodecyl mercaptan, etc., which are effective in reducing cross-linking in the copolymer. In general, the mercaptans should be used in concentrations of 0.1% to 5.0% by weight, based on the weight of polymerizable monomers present in the charge.

Alternatively the chlorine containing polymer may be prepared by chlorinating homopolymers or copolymers. For example chlorinated rubbers such as polychloroprene may be prepared by reacting a rubber with chlorine gas. In a similar manner chlorinated polyethylene may be prepared.

According to an alternative embodiment the heat converting substance may be contained in the oleophobic surface layer provided that said substance is homogeneously distributed therein.

The oleophobic surface layer in accordance with the present invention preferably has a thickness of at least 1.0µm and more preferably at least 1.5µm. The maximum thickness of the surface layer is not critical but will preferably be not more than 5µm and more preferably not more than 4µm. It has been found that the thickness of the oleophobic surface layer influences the printing endurance, sharpness and resolution of the printing plate.

According to the present invention the oleophobic surface layer is preferably cured and more preferably contains a hardened silicone coating. Preferably the silicone coating contains one or more components one of which is generally a linear silicone polymer terminated with a chemically reactive group at both ends and a multifunctional component as a hardening agent. The silicone coating can be hardened by condensation curing, addition curing or radiation curing.

Condensation curing can be performed by using a hydroxy terminated polysiloxane that can be cured with a multifunctional silane. Suitable silanes are e.g. acetoxy silanes, alkoxy silanes and silanes containing oxime functional groups. Generally the condensation curing is carried out in the presence of one or more catalyst such as e.g. tin salts or titanates. Alternatively hydroxy terminated polysiloxanes can be cured with a polyhydrosiloxane polymer in the presence of a catalyst e.g. dibutyltindiacetate.

Addition curing is based on the addition of Si-H to a double bond in the presence of a catalyst e.g. platinum. Silicone coatings that can be cured according to the addition curing thus comprise a vinyl group containing polymer, a catalyst e.g. chloroplatinic acid complexes and a polyhydrosiloxane e.g. polymethylhydrosiloxane. Suitable vinyl group containing polymers are e.g. vinyldimethyl terminated polydimethylsiloxanes and dimethylsiloxane/vinylmethyl siloxane copolymers.

Radiation cure coatings that can be used in accordance with the present invention are e.g. U.V. curable coatings containing polysiloxane polymers containing epoxy groups or electron beam curable coatings containing polysiloxane polymers containing (meth)acrylate groups. The latter coatings preferably also contain multifunctional (meth)acrylate monomers.

According to the present invention the ink repellant layer may comprise additional substances such as e.g. plasticizers, pigments, dyes etc..

According to the method of the present invention the heat mode recording material is image-wise exposed using a laser. Preferably used lasers are e.g. semiconductor lasers, YAG lasers e.g. Nd-YAG lasers, Argon lasers etc.. The laser may have a power output between 35 and 20,000mW and preferably operates in the infrared part of the spectrum. Preferably the support of the heat mode recording material is transparant and image-wise exposure proceeds through the support.

Subsequent to the image-wise exposure the heat mode recording element is developed in order to remove on the irradiated areas the oleophobic surface layer. Preferably said development is effected by rubbing said oleophobic surface layer. Rubbing can be done using e.g. a brush or a cotton pad. Rubbing of the heat mode recording material may be carried out in the presence of a solvent such a e.g. isopropanol, n.heptane or other hydrocarbon liquids when the surface layer contains a polysiloxane or more preferably in absence of a liquid. Rubbing according to the preferred modi operandi offers in addition to the ecological advantage printing plates of high resolution and sharpness.

The present invention will now be illustrated with the following examples without however limiting it thereto. All parts are by weight unless otherwise specified.

### EXAMPLE 1

The following coating solution for the ink repellant layer was prepared:

| | |
|---|---|
| iso-octane | to 1000ml |
| divinyl terminated dimethylpolysiloxane | 59.5g |
| dimethylpolysiloxane gum | 28.2g |
| divinyltetramethyl disiloxane complex of platinum | 0.37g |
| hydride terminated dimethylpolysiloxane (DC 7048 cross-linker from Dow) | 1.79g |
| stabilizer (Surfinol 61 from Air products) | 0.18g |

The following coating solution for the recording layer was prepared:

| | |
|---|---|
| ethylacetate/butylacetate (60:40)mixture | to 1000 ml |
| Spezial Schwartz (carbon black from Degussa) | 24.6 g |
| Solsperse 28000 (wetting agent from ICI) | 2.64 g |
| Solsperse 5000 (wetting agent from ICI) | 0.52 g |
| nitrocellulose | 11.87 g |
| Cymel 301 ( melamine hardener from Dyno Cytec) | 2.14 g |
| p-toluene sulphonic acid | 0.42 g |

A comparitive heat mode recording material A0 was prepared by coating the above coating solution for the recording layer to a polyethylene terephthalate film support (175µm) with a wet coat thickness of 22 µm to a dry layer thickness of 2.2 µm.

To this layer was coated the ink repellant layer from the above described coating solution to a dry thickness of 3.42 µm. Subsequent the ink repellant layer was cured for 3min. at 130°C.

Heat mode recording materials according to the invention were prepared similar to the comparative sample with the exception that or the back side of the flexible support was left as such, giving elements An, was coated with a back side solution B, giving elements Bn, with a back side solution C, giving elements Cn or with a back side solution D, giving elements Dn (whereby n stands for an integer from 0 to 3) and/or the coating solution for the ink repellant layer further contained no supplemental agent giving elements X0 or contained 100 mg/m² of matting agent 1, giving elements X1 or contained 100 mg/m² of matting agent 2, giving elements X2 or contained 100 mg/m² of matting agent 3, giving elements X3, X standing for A, B, C or D with these capitals having the meaning as mentioned above.

The back coating B contains 233 mg/m² gelatin, 520 mg/m² colloidal silica with a surface area of 300 m²/gr and 10 mg/m² of amorphous silica with a diameter of 4 µm.

The back coating C comprises PVA, TiO₂ and hydrolyzed tetraalkyl orthosilicate, wherein SiO₂ constitutes 7.5 weight % of the total weight of said matrix, TiO₂ constitutes 75 weight % of the total weight of said matrix and PVA constitutes 17.5 weight % of the total weight of said matrix. The total weight of said matrix amounts to 6.8 g/m².

The back coating D comprises 200 mg/m² of a polymethyl-methacrylate latex (particles diameter between 25 and 300 nm), 20 mg/m² colloidal silica with a surface area of 100 m²/gr, 10 mg/m² of a polyethylene wax, 7 mg/m² of polystyrene sulphonic acid, 3 mg/m² of poly(3,4-ethylenedioxy-thiophene) and 30 mg/m² of polymethyl-methacrylate matting agent with a diameter of 6 µm.

Matting agent 1 is amorphous silica with a weight average diameter between 4.3 and 5.3 µm, treated with an amide of a fatty acid (SYLOBLOC 250). Matting agent 2 is a wax-treated amorphous silica with a weight average diameter between 4.3 and 4.9 µm (SYLOID 7000). Matting agent 3 is an amorphous aluminosilicate with a weight average diameter of at most 40 µm (SYLOSIV A3). SYLOBLOC 250, SYLOID 7000 and SYLOSIV A3 are trade names from Grace Davison, Belgium.

The kinetic coefficient of friction (µₖ) and the blocking of the obtained heat mode recording materials were measured. µₖ was measured according to ASTM D1894. Blocking was measured by a visual inspection during roll-on of the film. Therefore a film with a width of 24 cm is rolled-on at a speed of 7 m/min. The mechanismus which steers the rolling-on of the film is displaced over 2 cm. The effect of this displacement on the rolled-on film is evaluated qualitatively.

| Evaluation | Result |
|---|---|
| 5 | heavy wrinkles |
| 4 | wrinkles |
| 3 | light wrinkles |
| 2 | no wrinkles, stiff recovery |
| 1 | no wrinkles, lightly stiff recovery |
| 0.5 | light effect |
| 0 | no effect |

The proofs are acceptable up to an evaluation of 2; proofs with an evaluation of 3 or more are not longer acceptable. The results for the various heat mode recording materials are given in table 1.

**Table 1**

| Material | µₖ | Blocking |
|---|---|---|
| A0 | 4.4 | 5 |
| B0 | 2.0 | 2 |
| C0 | 2.6 | 1 |
| D0 | 0.54 | 0.5 |
| B1 | 1.23 | 0 |
| B2 | 0.39 | 0 |
| B3 | 0.45 | 0 |
| D1 | 0.23 | 0 |
| D2 | 0.20 | 0 |
| D3 | 0.20 | 0 |

It is clear from these results that heat mode recording material A0 (comparison material) with a kinetic coefficient of friction of 4.4 showed very strong blocking while the other heat mode recording materials (materials according to the invention) showed an acceptable to none blocking. The best results are obtained when as well a back layer coating as a matting agent in the ink repellant layer are used.

## Claims

1. A heat mode recording material comprising on a flexible support having an oleophilic surface (i) a recording layer containing a light-to-heat converting substance capable of converting radiation into heat and (ii) an oleophobic surface layer, wherein said oleophobic surface layer and said recording layer may be the same layer, **characterized in that** the recording material comprises a back side coating and/or that a matting agent is present in the oleophobic surface layer, and further **characterized in that** the kinetic coefficient of friction (µₖ ) of said material when sliding one side of said material over the other side of said material is not more than 2.6.

2. A heat mode recording material according to claim 1 wherein said kinetic coefficient of friction is comprised between 1.25 and 0.05.

3. A heat mode recording material according to claim 1 wherein said back side coating contains between 175 and 750 mg/m² of gelatin, between 50 and 1000 mg/m² of colloidal silica with a surface area of at least 100 m²/gr and between 1 and 100 mg/m² of amorphous silica.

4. A heat mode recording material according to claim 1 wherein said back side coating comprises between 100 and 500 mg/m² of a polymethyl-methacrylate latex, between 5 and 50 mg/m² of colloidal silica with a surface area of at least 100 m²/gr, between 3 and 30 mg/m² of a polyethylene wax, between 3.1 and 12 mg/m² of polystyrene sulphonic acid, between 0.9 and 4 mg/m² of poly(3,4-ethylenedioxythiophene) and between 10 and 100 mg/m² of polymethyl-methacrylate matting agent.

5. A heat mode recording material according to claim 1 wherein said back side coating comprises PVA, TiO₂ and hydrolyzed tetraalkyl orthosilicate, wherein SiO₂ constitutes between 7 and 30 weight % of the total weight of said matrix, TiO₂ constitutes between 63 and 83 weight % of the total weight of said matrix and PVA constitutes between 7 and 30 weight % of the total weight of said matrix, the total weight of said matrix lying between 5 and 10 g/m².

6. A heat mode recording material according to claim 1 wherein said matting agent is an inorganic compound.

7. A method for making a lithographic printing plate requiring no dampening liquid comprising the steps of:
- image-wise exposing by means of a laser beam a heat mode recording material according to any of claims 1 to 6
- developing the exposed heat mode recording material thereby removing said oleophobic surface layer in the exposed areas so that the underlying oleophilic surface is exposed.

8. A method for making a lithographic printing plate requiring no dampening liquid in accordance with claim 7 wherein said development is effected by rubbing said oleophobic surface layer in the presence of a liquid or in absence of a liquid.

## Patentansprüche

1. Ein wärmeempfindliches Aufzeichnungsmaterial, das auf einem biegsamen Träger mit einer oleophilen Oberfläche (i) eine Aufzeichnungsschicht mit einer Licht in Wärme umwandelnden Substanz, die Strahlung in Wärme umzuwandeln vermag, und (ii) eine oleophobe Oberflächenschicht enthält, wobei die oleophobe Oberflächenschicht und die Aufzeichnungsschicht ein und dieselbe Schicht sein können, **dadurch gekennzeichnet, daß** die Rückseite des Aufzeichnungsmaterials beschichtet ist und/oder die oleophobe Oberflächenschicht ein Mattiermittel enthält und weiterhin **dadurch gekennzeichnet, daß** eine der kinetische Reibungskoeffizient (µₖ) des Materials nicht mehr als 2,6 beträgt, wenn eine Seite des Materials über die andere Seite des Materials gleitet.

2. Wärmeempfindliches Aufzeichnungsmaterial nach Anspruch 1, **dadurch gekennzeichnet, daß** der kinetische Reibungskoeffizient zwischen 1,25 und 0,05 liegt.

3. Wärmeempfindliches Aufzeichnungsmaterial nach Anspruch 1, **dadurch gekennzeichnet, daß** die Rückseitenbeschichtung Gelatine in einem Verhältnis zwischen 175 und 750 mg/m², kolloidale Kieselsäure mit einer spezifischen Oberfläche von zumindest 100 m²/g in einem Verhältnis zwischen 50 und 1.000 mg/m² und amorfe Kieselsäure in einem Verhältnis zwischen 1 und 100 mg/m² enthält.

4. Wärmeempfindliches Aufzeichnungsmaterial nach Anspruch 1, **dadurch gekennzeichnet, daß** die Rückseitenbeschichtung einen Polymethylmethacrylatlatex in einem Verhältnis zwischen 100 und 500 mg/m², kolloidale Kieselsäure mit einer spezifischen Oberfläche von zumindest 100 m²/g in einem Verhältnis zwischen 5 und 50 mg/m², ein Polyethylenwachs in einem Verhältnis zwischen 3 und 30 mg/m², Polystyrolsulfonsäure in einem Verhältnis zwischen 3,1 und 12 mg/m², Poly(3,4-ethylendioxythiophen) in einem Verhältnis zwischen 0,9 und 4 mg/m² und Polymethylmethacrylat-Mattiermittel in einem Verhältnis zwischen 10 und 100 mg/m² enthält.

5. Wärmeempfindliches Aufzeichnungsmaterial nach Anspruch 1, **dadurch gekennzeichnet, daß** die Rückseitenbeschichtung PVA, TiO₂ und hydrolysiertes Tetraalkylorthosilikat enthält, wobei SiO₂ in einem Verhältnis zwischen 7 und 30 Gew.-%, bezogen auf das Gesamtgewicht der Matrix, TiO₂ in einem Verhältnis zwischen 63 und 83 Gew.-%, bezogen auf das Gesamtgewicht der Matrix, und PVA in einem Verhältnis zwischen 7 und 30 Gew.-%, bezogen auf das Gesamtgewicht der Matrix, enthalten ist, wobei das Gesamtgewicht der Matrix zwischen 5 und 10 g/m² liegt.

6. Wärmeempfindliches Aufzeichnungsmaterial nach Anspruch 1, **dadurch gekennzeichnet, daß** das Mattiermittel eine anorganische Verbindung ist.

7. Ein durch die nachstehenden Schritte **gekennzeichnetes** Verfahren zur Herstellung einer lithografischen Druckplatte, in dem kein Anfeuchtwasser benötigt wird :
- bildmäßige Belichtung mit Laserstrahlung eines wärmeempfindlichen Aufzeichnungsmaterials nach einem der Ansprüche 1 bis 6,
- Entwicklung des belichteten wärmeempfindlichen Aufzeichnungsmaterials, wobei die oleophobe Oberflächenschicht in den belichteten Bereichen entfernt und dadurch die unterliegende oleophile Oberfläche freigelegt wird.

8. Ein Verfahren zur Herstellung einer kein Anfeuchtwasser benötigenden lithografischen Druckplatte nach Anspruch 7, **dadurch gekennzeichnet, daß** die Entwicklung durch Abwischen der oleophoben Oberflächenschicht in Gegenwart von einer Flüssigkeit oder in Abwesenheit einer Flüssigkeit vorgenommen wird.

## Revendications

1. Matériau d'enregistrement thermosensible comprenant, sur un support flexible possédant une surface oléophile, (i) une couche d'enregistrement contenant une substance de transformation de la lumière en chaleur capable de transformer un rayonnement en chaleur et (ii) une couche superficielle oléophobe, dans lequel ladite couche superficielle oléophobe et ladite couche d'enregistrement peuvent représenter la même couche, **caractérisé en ce que** le matériau d'enregistrement comprend une couche dorsale et/ou **en ce que** l'agent de matage est présent dans la couche superficielle oléophobe, est **caractérisé en outre en ce que** le coefficient cinétique de friction (µₖ) dudit matériau, lorsqu'on fait glisser un côté dudit matériau par-dessus l'autre côté dudit matériau, n'est pas supérieur à 2,6.

2. Matériau d'enregistrement thermosensible selon la revendication 1, dans lequel ledit coefficient cinétique de friction est compris entre 1,25 et 0,05.

3. Matériau d'enregistrement thermosensible selon la revendication 1, dans lequel ladite couche dorsale contient de la gélatine à concurrence d'une valeur entre 175 et 750 mg/m², de la silice colloïdale à concurrence d'une valeur entre 50 et 1000 mg/m² possédant une aire de surface d'au moins 100 mg/g et de la silice amorphe à concurrence d'une valeur entre un et 100 mg/m².

4. Matériau d'enregistrement thermosensible selon la revendication 1, dans lequel ladite couche dorsale comprend un latex de polyméthacrylate de méthyle à concurrence d'une valeur entre 100 et 500 mg/m², de la silice colloïdale possédant une aire de surface d'au moins 100 m²/g à concurrence d'une valeur entre 5 et 50 mg/m², une cire de polyéthylène à concurrence d'une valeur entre 3 et 30 mg/m², de l'acide polystyrènesulfonique à concurrence d'une valeur entre 3,1 et 12 mg/m², du poly(3,4-éthylidènedioxythiophène) à concurrence d'une valeur entre 0,9 et 4 mg/m² et un agent de matage à base de polyméthacrylate de méthyle à concurrence d'une valeur entre 10 et 100 mg/m².

5. Matériau d'enregistrement thermosensible selon la revendication 1, dans lequel ladite couche dorsale comprend du PVA, du dioxyde de titane et de l'orthosilicate de tétraalkyle hydrolysé, du dioxyde de silicium représentant entre 7 et 30 % en poids du poids total de ladite matrice, le dioxyde de titane représentent entre 63 et 83 % en poids du poids total de ladite matrice et le PVA représentant entre 7 et 30 % en poids du poids total de ladite matrice, le poids total de ladite matrice se situant entre 5 et 10 g/m²

6. Matériau d'enregistrement thermosensible selon la revendication 1, dans lequel ledit agent de matage est un composé inorganique.

7. Procédé pour fabriquer un cliché d'impression lithographique, qui n'a pas besoin de liquide de mouillage, comprenant les étapes consistant à
- exposer en forme d'image à l'aide d'un faisceau laser, un matériau d'enregistrement thermosensible selon l'une quelconque des revendications 1 à 6 ;
- développer le matériau d'enregistrement thermosensible exposé pour ainsi éliminer ladite couche superficielle oléophobe dans les zones exposées de façon à exposer la surface oléophile sous-jacente.

8. Procédé de fabrication d'un cliché d'impression lithographique, qui n'a pas besoin de liquide de mouillage, selon la revendication 7, dans lequel on procède audit développement par friction de ladite couche superficielle oléophobe en présence d'un liquide ou en l'absence d'un liquide.
